

Nov. 4, 1941.

A. H. BATCHELDER

2,261,577

MULTIPHASE LUBRICATING SYSTEM

Filed April 17, 1939

2 Sheets-Sheet 1



Fig. 1



Fig. 2



Fig. 3



Fig. 4



Fig. 5

Augustus H. Batchelder  
INVENTOR

By *[Signature]*  
ATTORNEYS

Nov. 4, 1941.

A. H. BATCHELDER

2,261,577

MULTIPHASE LUBRICATING SYSTEM

Filed April 17, 1939

2 Sheets-Sheet 2

Fig. 6



Augustus H. Batchelder

INVENTOR

BY J. Nakama  
ATTORNEYS

## UNITED STATES PATENT OFFICE

2,261,577

## MULTIPHASE LUBRICATING SYSTEM

Augustus H. Batchelder, Berkeley, Calif., assignor  
to Standard Oil Company of California, San  
Francisco, Calif., a corporation of Delaware

Application April 17, 1939, Serial No. 268,312

16 Claims. (Cl. 252—56)

This invention relates to a multiphase lubricating system, and more particularly to a lubricating system or composition comprising a lubricating oil phase and one or more additional phases.

An object of the invention is to provide a useful lubricating system or composition having certain novel characteristics.

A further object is to provide a lubricating medium having a negligible viscosity-temperature coefficient over temperature ranges in the order of at least approximately 50° F. and as great as 100° F. or more.

An additional object of the invention is to provide a lubricating composition which will show substantially no loss of viscosity when the temperature thereof is raised from approximately 200° to approximately 300° F.

Another object comprises the production of a novel type of multiphase lubricating composition, an oil phase and a continuous phase other than said oil phase containing a high molecular weight organic resinous material dispersed therein.

A still further object of the invention is the provision of a novel method for maintaining the viscosity of a lubricant substantially constant over relatively wide temperature ranges.

It is also an object of the invention to furnish an apparatus suitable for effecting lubrication with the multiphase system here disclosed and for carrying out the process of the invention.

Additional objects will be apparent from the detailed description of the invention hereinafter given.

Lubricating compositions containing viscous materials have been proposed heretofore; for example, viscous materials have been dissolved in lubricating oils in order to enhance the viscosity index of the resulting solution (the term "viscosity index" is defined by Dean and Davis in "Chemical & Metallurgical Engineering," vol. 36, pp. 618-619). In such prior known compositions the viscous material has been in solution in the oil and separation of the addition agent as an independent phase has been carefully avoided as undesirable. The increase in viscosity index of these types of solutions was effected by initially imparting to the oil a large increase in viscosity at normal atmospheric temperatures, which increase resulted in a flattening of the viscosity-temperature curve. This initial increase in viscosity represented the total increase to be obtained and was not later multiplied or increased at elevated temperatures.

Although such an expedient has given some im-

15 oils, it has not been possible with these solutions to produce compositions having constant viscosities over substantial temperature ranges such as 50° or 100° F. Further, the large initial increase in viscosity obtained by solution of the viscous material in the oil at ordinary atmospheric temperatures, in some instances necessitates the use of a lighter oil as the base stock for the lubricant in order to avoid an unduly high viscosity at lower temperatures and to meet the viscosity specifications for a given grade of oil. This lighter base oil is consequently more volatile than heavier oils which would be used except for the presence of the addition agent, and such increased volatility tends to cause greater oil consumption and may largely offset advantages presumed to result from the higher viscosity index.

15 I am also aware that various insoluble materials have been dispersed in lubricating oils to enhance the lubricating action thereof; for instance, materials such as graphite, extreme pressure addition agents like lead sulfide, and drying oil polymers which remain insoluble in the particular base oil used even at elevated temperatures, have been proposed. These materials, by reason of their insolubility in the oil, have reduced the viscosity-temperature coefficient of the lubricating oil only to a minor or unappreciated degree, if at all.

20 30 It will be noted that the above described prior art compositions are characterized by a dispersed material which is either entirely soluble in the oil at ordinary temperatures, such as 65° to 100° F., or which is substantially entirely insoluble in the lubricating oil not only at these temperatures but also at elevated temperatures, such as from 200° to 300° F. The present invention is concerned with a different type of lubricating composition or system and is not to be confused therewith.

25 35 I have discovered that lubricating compositions having negligible viscosity-temperature coefficients (viscosity-temperature coefficient is the slope of the viscosity-temperature curve)—i. e., negligible change of viscosity with change of temperature—may be obtained by utilizing a multiphase system.

30 35 According to the invention a first phase comprises a lubricating oil, a second phase comprises a high molecular weight organic resinous material and the two phases have certain solubility relationships. The phases comprising the components of my invention may be separately new or old, since it is the novel combination of components which I regard as the primary feature

of my invention rather than the composition of the independent components.

The lubricating oil phase of my composition may comprise a mineral lubricating oil; a vegetable or animal oil; or a synthetic lubricant such as liquid, olefine polymers; hydrogenated, liquid olefine polymers; or other synthetic hydrocarbons having a viscosity in the range normally utilized as lubricating oils. The second phase of my composition contains a high molecular weight resinous material which is highly viscous and preferably one characterized by long molecules such as are obtained by chain reactions of the polymerization or condensation type.

Although there are a number of types of multiphase systems which may be utilized to accomplish the objects of this invention, one common property of the systems which characterizes the invention is the provision of a separate phase which tends to dissolve into the lubricating oil at high temperatures, such as 200° to 300° F., and which is substantially insoluble in the oil, and hence goes out of solution at ordinary temperatures, such as 65° to 100° F. This second phase may be said to be "temperature-sensitive" in that it tends to dissolve or disappear at high temperatures and precipitate or reappear at low temperatures.

Various of the different types of multiphase systems are illustrated in the drawings in which:

Figure I is a diagrammatic illustration of a two-phase system and an apparatus for contacting the phases to maintain them substantially in equilibrium.

Figure II represents a diagrammatic magnified view of a composition in which particles of the phase containing organic resinous material are dispersed in the oil phase. The dispersed particles represented are of greater than colloidal size.

Figure III diagrammatically illustrates a multiphase system and an apparatus for maintaining equilibrium between the several phases.

Figure IV represents a two-phase system in which one phase may be a colloidal solution or suspension in a dispersing medium other than the lubricating oil.

Figure V shows a diagrammatic and magnified view of a colloidal phase dispersed in an oil phase and in which the dispersing medium for the colloidal phase comprises particles of greater than colloidal size.

Figure VI gives curves showing the viscosity-temperature characteristics of compositions utilizing the present invention.

As described hereinabove, one phase comprises a lubricating oil which may be an oil of various types, e. g., mineral oil, vegetable or animal oils, and the synthetic hydrocarbons. The second phase of the multiphase system of this invention may be one of several different types as exemplified by the following:

(1) A resinous material largely insoluble in the oil at ordinary atmospheric temperatures, for instance, less than 0.1% soluble at 65° or 100° F. and largely soluble in the oil at elevated temperatures as, for example, more than 1% soluble at 200° or 300° F.

(2) A high molecular weight organic resinous material which itself may not have the above solubility characteristics. However, in this variation the second phase comprises a solution of the resinous material in which the solvent is substantially non-volatile and may be either (a) immiscible with the oil even at elevated tempera-

tures or (b) immiscible with the oil at ordinary temperatures (65° to 100° F.) but substantially miscible at elevated temperatures (200° to 300° F.). Where the solvent is immiscible as in (a), it is of course essential that the oil solubility of the dissolved resinous material be such that the resinous material will remain dissolved in the solvent phase in the low temperature range but will increase in solubility in the oil as the temperature rises, to the extent that said material will pass from the solvent phase to the oil phase. The resinous material may pass into and out of solution in the oil, as the temperature varies, either by reason of variations in solubility of the material alone or by reason of the solvent dissolving in the oil and carrying with it the resinous material, or because both the solvent and the resin become more soluble in the oil.

(3) Analogous to the second variation above-described, the second phase may comprise a colloidal dispersion, i. e. an emulsion or colloidal suspension in a "solvent" or dispersing medium other than the lubricating oil. The colloidally dispersed resinous material may thus pass from colloidal dispersion in the "solvent" to solution in the oil as the temperature rises and then return to colloidal dispersion in the "solvent" as the temperature is again lowered.

(4) In combination with any of the above three systems, a third component may be introduced which decreases the viscosity of the oil when the component is dissolved therein and which goes out of solution at elevated temperature and into solution in the oil at ordinary temperatures. A suitable type of third component comprises a relatively volatile material which passes out of solution at elevated temperatures as a vapor phase and then goes back into solution in the oil either directly as a vapor phase or after forming an intermediate liquid phase when the temperature is lowered. This type of system may therefore involve either three or four phases, namely: the lubricating oil phase, the second liquid phase containing resinous material, the vapor phase of the third component, and a liquid phase comprising said third component.

This third component may advantageously be of the type which, when dissolved in the oil at low temperature, tends to force the resinous material from solution in the oil into the separate second phase. Low molecular weight acyclic hydrocarbons, such as propane, butane, pentane, and hexane, have this additional effect on certain resinous materials.

The drawings serve to illustrate and explain the operation of representative types of systems utilizing this invention. In Figure I the first phase 1, comprising lubricating oil, and the second phase 2 are held in container 3 provided with a baffle 4, inlet 5, and outlet 6. Phase 2 contains a high molecular weight organic material having solubility characteristics such that a substantial amount of the material goes into solution in the oil when the latter is at elevated temperatures and which goes out of solution at ordinary temperatures. A desirable material will be less than 0.1% soluble at 65° F., more than 2% soluble at 300° F., and possess a viscosity in the order of 146,000 times that of the lubricating oil (viscosity being measured in centipoises). These two phases are maintained in equilibrium by the oil flowing from inlet 5 into the container around baffle 4 in contact with phase 2 to the outlet 6. Phase 2 may comprise a high molecular weight normally liquid resinous material or a resinous

material which is either normally liquid or normally solid, but dissolved in a solvent as hereinabove described.

Figure II shows a magnified view diagrammatically illustrating a composition comprising the same types of components as in Figure I. However, in Figure II the second phase 8 is a discontinuous one undissolved in the oil 7 at low temperatures, but non-colloidally dispersed therein. The discontinuous phase may be maintained in dispersion by means of colloidal or non-colloidal peptizing agents, e. g. soaps. By "non-colloidal" I mean that the dispersed particles are of greater than colloidal size and do not exhibit Brownian movement. In general, particles of a size greater than in the order of 0.1 mu (0.0001 mm.) are non-colloidal. The viscosity of this combination is maintained substantially constant through the following cycle of operations: Assume the system at equilibrium at 100° F.; less than the approximately 0.1% of the organic resinous material by weight based on the oil will be dissolved. Substantially all of the resinous material will therefore be in the dispersed phase 8 and, in small proportions in the order of 2%, it will not greatly increase the viscosity of the lubricant. The viscosity of the system may therefore approximate the normal viscosity of the oil alone at 100° F. As the temperature of the composition is raised to 300° F., the dispersed phase 8 dissolves in the oil 7, increasing the viscosity thereof in an amount sufficient substantially to offset the decrease in viscosity of the oil, which normally would occur with the rise in temperature. Hence, at 300° F. all of the dispersed phase 8 may be dissolved in the oil 7, and the viscosity of the lubricant may be equal to or even greater than that of the lubricant at 100° F. When the temperature is lowered, the reverse effect obtains and the resinous material precipitates out of solution in the oil, thereby decreasing the viscosity of the lubricant to offset the normal increase produced by the lowered temperature.

Figure III illustrates a closed lubricating system comprising an oil phase 9, a second liquid phase 10 lighter than oil and containing an organic resinous material, a third component 11 which may be in liquid phase at 16 at low temperatures and in vapor phase 12 the pressure of which will vary with temperature. Container 13 and its appurtenances are adapted to maintain this multiphase system in substantial equilibrium. Inlet 14 and outlet 15 are provided for admitting lubricant 9 and removing it from container 13. In the container the oil phase is contacted with liquid phase 10 as well as with the third component at 16. The oil phase is also in equilibrium with the vapor phase 12.

A check valve 17 is provided on closed container 13 to prevent pressure in the container from rising above predetermined limits. A suitable form of valve comprises ball 18 resting on valve seat 19 and held in position thereon by spring 20. Orifice 21 affords means for the escape of vapor phase 12 when the pressure thereof becomes greater than the predetermined load on ball 18 exerted by spring 20.

Container 22 is provided for holding liquid phase 11 and is connected to container 13 by means of conduit 24 provided with valve 29, which is normally open and allows liquid 11 to flow freely into and out of container 13 as the liquid is dissolved in or precipitated out of oil phase 9. A float 25 is connected to valve 29 through linkage 26 and serves to close said valve

when the level of liquid 11 reaches a predetermined height and thereby prevents overflow. A second conduit 28 affords means for allowing liquid 11 to flow into container 13, but a check valve 27 prevents flow of fluid from container 13 to container 22.

A cycle of operation of the system of Figure III is as follows: Assume the system to be at equilibrium at a temperature T<sub>1</sub>, e. g. at 100° F., 10 at which temperature the solubility of phase 10 in the oil is negligible and phase 10 thereby does not substantially increase the viscosity of the oil at T<sub>1</sub>. Liquid 11 is substantially soluble in oil at T<sub>1</sub>, but also may appear in vapor phase 12, 15 having a partial pressure P<sub>1</sub>. The effect of liquid 11 being dissolved in the oil is to lower the viscosity of phase 9 below that which the lubricating oil alone would possess at T<sub>1</sub>.

When the temperature rises to T<sub>2</sub>, e. g. 200° to 20 300° F., the viscosity of the oil alone decreases greatly, but phase 10 comprising an organic resinous material, substantially soluble in the oil at this temperature, imparts increased viscosity to the oil by reason of its solubility therein, to the extent that the viscosity of the solution, even though still predominantly lubricating oil, is comparable to the viscosity of phase 9 at T<sub>1</sub>. Actually, the viscosity of the solution at T<sub>2</sub> may be equal to or even greater than that of phase 9 at 25 T<sub>1</sub>. Further, by reason of the increase in temperature, the solubility of component 11 is greatly decreased and this component goes out of solution as vapor phase at 12. In some cases the component may also form a separate liquid phase 30 at 16, depending upon pressures and temperatures. Release of component 11 from solution further serves to increase the viscosity of lubricating phase 9 and serves to enhance the action of phase 10 in maintaining the viscosity of phase 40 9 substantially constant. In some instances the removal of component 11 from solution into vapor phase 12 and/or liquid phase 16 may also serve to enhance the solubility of phase 10 in phase 9, thereby further magnifying the compensating effect on viscosity.

To complete the cycle, assume that after the system has reached equilibrium at T<sub>2</sub>, the temperature is again reduced to T<sub>1</sub>. The high molecular weight resinous material dissolved from phase 10 at T<sub>2</sub> precipitates out of solution as the temperature is lowered and returns to phase 10, 50 thereby decreasing the viscosity of phase 9 and compensating for the normal increase produced by lower temperatures. Component 11 also becomes more soluble in the oil, dissolves therein as the temperature is lowered, and tends to reduce the viscosity of the oil. Thus, although the viscosity of phase 9 tends to increase as the temperature is lowered, this effect is offset by the 55 passage of one component from solution to phase 10 and passage of phases 12 and 16 back into solution.

In the above description the effect of variation of pressure in vapor phase 12 has not been discussed. At T<sub>1</sub> phase 12 has a lower pressure P<sub>1</sub>. At T<sub>2</sub> the pressure will be substantially greater, assuming that the volume of phase 12 remains substantially constant or does not increase proportionally to the absolute temperature. Initial increase in the pressure of phase 12 may be taken up by expansion of this gas phase to force liquid phase 16 back into container 22. The amount of liquid which may be forced into container 22 is definitely limited by float 25, 70 which closes valve 29 at a predetermined level

in container 22. As the temperature continues to rise, additional increase of pressure may be released through valve 17 until such time as equilibrium is reached at  $T_2$ . After equilibrium has been reached, the temperature may again be reduced to  $T_1$  and pressure in phase 12 will accordingly drop to  $P_1$ . This results in a partial vacuum and, since valve 29 is retained in closed position by the elevated level of fluid 11 in container 22, it is necessary to effect return of component 11 to container 13 through conduit 28. Check valve 27 in conduit 28 permits such return. Fluid 11 flows through conduit 28 to container 13 until sufficient quantity is dissolved in the oil to reduce the level in container 22 and open valve 29, thereby allowing free communication between containers 22 and 13 through conduit 24.

Figure IV illustrates a system analogous to that of Figure I, the principal difference being that phase 35 comprises a colloidal dispersion of a high molecular weight organic resinous material in a continuous phase of high boiling liquid which, like the solvent hereinabove described, is immiscible with the lubricating oil at ordinary temperatures and may or may not vary substantially in oil solubility as the temperature rises. In this figure container 30, provided with inlet 31, outlet 32, and baffle 33, holds the lubricating oil phase 34 and the colloidal phase 35. The dispersed material in phase 35 may be either normally solid, normally plastic, or normally liquid. This dispersion should have the solubility characteristics previously described with respect to phases 2 and 8 in Figures I and II. Thus, at high temperatures the material dispersed in phase 35, either independently or together with the dispersing medium, will become substantially soluble in the oil, dissolve therein, and maintain the viscosity within the range desired. A filter 36 is provided for removing undissolved material from the oil phase as it passes from outlet 32 to oil feed pipe 37.

Figure V shows a system analogous to that of Figure II and comprises a discontinuous phase 39 undissolved and non-colloidal dispersed in oil phase 38. Discontinuous phase 39 comprises particles of greater than colloidal size. These particles are composed of a high boiling liquid dispersing medium which is immiscible with the lubricating oil at ordinary temperatures, and may or may not vary substantially in oil solubility as the temperature rises. This high boiling dispersing medium contains a high molecular weight resinous material in a colloidal state of dispersion. Thus a colloidal dispersion in a liquid medium other than the oil phase is non-colloidal dispersed as a discontinuous phase in the continuous oil phase. The dispersion in the discontinuous phase should have the solubility characteristics previously described with respect to phases 2 and 8 in Figures I and II. At high temperatures the material dispersed in phase 39, either independently or together with the dispersing medium of that phase, will become substantially soluble in the oil, dissolve therein, and maintain the viscosity within the range desired. Conversely, as the temperature is lowered the dissolved material will precipitate out of the oil into the discontinuous colloidal phase thereby compensating for viscosity changes occurring as the oil is cooled.

The following examples and data on the viscosities of specific lubricating compositions utilizing the principles of this invention are given for 75

purposes of illustration and to guide those skilled in the art in the practice of the invention:

A two-phase mixture comprising lard oil as a continuous phase and a rubber-like highly polymerized olefin as a discontinuous phase non-colloidal dispersed therein was prepared. The discontinuous phase was substantially insoluble in the oil at ordinary temperatures and therefore existed as a separate phase under such conditions. The viscosity-temperature curves of 1%, 2% and 5% of the olefin polymer are shown in Figure VI. Attention is particularly directed to the following comparative viscosities of the lubricating oil per se and the two-phase lubricant:

| 20     | Weight per cent of polymer | Viscosity in centipoises at |      |
|--------|----------------------------|-----------------------------|------|
|        |                            | 210° F. 300° F.             |      |
|        |                            | 7.4                         | 3.36 |
| 0..... | 10.....                    | 7.4                         | 3.36 |
| 2..... | 10.....                    | 10                          | 9.8  |

It will be observed that the viscosity of the single phase lubricant decreased approximately 44% as the temperature was raised from 210° F. to 300° F., whereas the viscosity of the two-phase lubricant was altered only a negligible amount. Further, the lard oil used as a basis of comparison had a viscosity index of 143 which, it will be noted, is extremely high. The difference between the viscosity-temperature coefficient of the two-phase lubricants tested and an ordinary mineral oil would, therefore, be much greater than the differences illustrated here.

Alternative compositions which give analogous results comprise: (1) a lubricating oil phase such as castor oil, other vegetable oils, or animal oils, and a second phase of a high molecular weight iso-butene polymer; (2) a heavy linseed oil polymer of a jelled or semi-solid consistency, soluble at elevated temperatures such as 200-300° F. and insoluble at ordinary temperatures, dispersed as a discontinuous phase in mineral oil of a suitable solvent power. In straight mineral oil, solvency and viscosity index are related and it has been found that, in general, to obtain proper correlation between the solubility of these last two phases the mineral oil should have a viscosity index above approximately 50. Hydrocarbon oils prepared by polymerization of mixed butenes, with or without hydrogenation, may be substituted for the mineral oil in this combination.

The invention is not limited to the specific examples herein given, but comprehends the broad combination of a plurality of phases in a lubricating composition wherein the solubility characteristics of the phases are correlated as hereinbefore described. In order for the lubricant to have a substantially constant viscosity over a given temperature range, the solubility of the resinous phase in the oil phase should be such that:

$$65 \quad \frac{dC}{dT}$$

should approximate

$$70 \quad \frac{1}{k} \cdot \frac{d(\log_e V)}{dT}$$

or, at any given temperature  $T$  within the range under consideration,  $C$  should approximate

$$\frac{1}{k} \log_e V + a$$

In the above, C is the weight fraction of resinous material dissolved in the oil;

$$\frac{dC}{dT}$$

is the change in said weight fraction with change in temperature; V is the viscosity of the lubricating oil; a is a constant of integration; and k is equal to the antilogarithm to the base e of

$$\frac{1}{C} \cdot \log \frac{V_1}{V_0}$$

where  $V_1$  is the viscosity of the oil and  $V_0$  the viscosity of the oil solution containing weight fraction C of the resin at a given temperature within the range being considered.

The high molecular weight organic resinous materials having solubility characteristics required for this invention may be selected from reaction products produced by various known polymerization and/or condensation reactions. The solubility of these reaction products may be adjusted to meet specific requirements by various expedients. For example, the oil solubility may be increased by introducing hydrocarbon radicals, as by alkylation of a resin-forming constituent before polymerization or condensation, or in some instances by alkylation during or after resinification. An example of this expedient comprises alkylation of phenol before condensation with formaldehyde to obtain a phenol formaldehyde resin. Conversely, when the reaction product is too soluble in the oil phase the solubility of this product may be decreased to the desired value by introducing oxygen, sulfur, nitro, amino, or other polar groups into the molecule, as by partial oxidation or sulfurization of a resin-forming constituent before, during or after resinification. An example of this procedure comprises blowing or sulfurizing a drying oil during polymerization by heating.

The following are mentioned as examples of the many types of materials and reaction products from which the organic resinous phase may be selected and the solubility thereof correlated with the particular lubricating oil phase to obtain the results herein disclosed: polymerized styrene, hydrogenated polymerized styrene, polymerized indene, hydrogenated polymerized di-olefins, such as hydrogenated polymerized butadiene or isoprene, or polymerization products of mono-olefins, such as isobutylene, isohexane, or of terpenes, cyclohexene or tetrahydronaphthalene, polymerized esters of unsaturated acids, preferably those in a highly polymerized state such as obtained in the presence of a catalyst. Polymers of vinyl esters, ethers and ketones may also be utilized. Resins formed by reaction of an alkyl dihalide with an aromatic hydrocarbon, such as ethylene dichloride with benzol, resins from alkylated phenol and formaldehyde, condensation products of oxygen-containing aliphatic materials of the class of esters, ethers, acids, alcohols and ketones containing unsaturated carbon-to-carbon bonds such as esters of acrylic acid, as well as resinous materials formed by condensation of naphthalene, anthracene, diphenyl, with an aldehyde followed by condensation with a long chain chlorinated hydrocarbon, comprise suitable high molecular weight resinous materials from which to select a phase of the composition herein disclosed. The above listed condensation or polymerization products may be formed with the assistance of condensation and polymerization

agents such as aluminum chloride, zinc chloride, boron fluoride and the like.

As examples of low molecular weight fluid materials which may be utilized for reducing viscosity of the oil at low temperatures and which will go out of solution from the oil as a vapor phase at high temperatures, the following are given: acetone, acetone, diethyl ketone, propyl alcohol, butyl alcohol, butyl chloride, amyl chloride, benzene, toluene, xylene, pentane, hexane, heptane, octane, cyclopentane, cyclohexane, cycloheptane, carbon disulfide, carbon tetrachloride, chloroform, dichloroethane, and the like. Where inflammability is to be avoided, fluids which are themselves unflammable may be utilized or may be mixed with normally inflammable fluids to decrease or avoid inflammability. Such a fluid is carbon tetrachloride.

From the disclosure hereinbefore given it will be apparent that the method of this invention comprises, broadly, contacting a lubricating oil phase with a second phase capable of going out of and into solution in the oil substantially to offset viscosity changes of the oil with alteration of temperature. More specifically, the method comprises maintaining a lubricating oil phase in contact with a second phase containing a high molecular weight resinous material, dissolving the resinous material in the oil phase as temperature rises, precipitating the resinous material from the oil phase to the resin phase as temperature lowers, and thereby maintaining the viscosity of the lubricating oil within predetermined limits.

By "high molecular weight resinous material" or "high molecular weight organic resinous material," wherever used herein, I intend to designate a normally viscous or plastic or solid material having carbon-containing molecules of high molecular weight. In general, the resinous material should have a viscosity of at least approximately 1,000 times that of the lubricating oil phase and preferably a viscosity in the order of 10,000 to 30,000, or more, times that of the lubricating oil phase—viscosity being measured for the purposes of this ratio in centipoises. When butene polymers are utilized as the high molecular weight material the polymer should have a molecular weight greater than 2,000, and preferably in the order of 10,000.

By "non-colloidal phase" or "macroscopic phase" I mean to designate a phase which is present either as an independent continuous phase having defined boundaries or as an undissolved dispersion in which the dispersed particles are of greater than colloidal size. A macroscopic dispersion, such as utilized herein, is characterized by dispersed particles containing at least thousands of molecules and is of a type different from solutions which are characterized by dispersed particles approaching unimolecular size.

The lubricating oil composition of this invention may contain, in addition to the resinous phase, compounding ingredients such as oiliness agents, extreme pressure addition agents, oxidation inhibitors, color stabilizers, anti-sludging agents, anti-piston ring sticking agents, pour point lowering agents, dyes or blooming agents and the like. It will also be apparent that the principle of this invention is applicable to lubricating compositions containing metal soaps either in grease-forming proportions or in proportions insufficient to form greases, as for example in gear oils or mineral castor machine oils.

While the character of the invention has been described in detail and numerous examples given,

this has been done by way of illustration only and with the intention that no limitation should be imposed upon the invention thereby. It will be apparent to those skilled in the art that numerous modifications and variations of the illustrative examples may be effected in the practice of the invention, which is of the scope of the claims appended hereto.

I claim:

1. A lubricant comprising a lubricating oil phase and a high molecular weight resinous phase, said resinous phase being substantially insoluble in the lubricating oil phase when cold and substantially soluble therein when hot, whereby said resinous phase goes out of and into solution in said oil phase with alteration of temperature to compensate for viscosity changes which would normally occur in said oil phase in the absence of said resinous phase.

2. A lubricant comprising a lubricating oil phase and a high molecular weight resinous phase, said resinous phase being substantially insoluble in the lubricating oil phase at a temperature within the range of approximately 65° F. to 100° F. and substantially soluble therein at a temperature within the range of approximately 200° to 300° F., whereby said resinous phase goes out of and into solution in said oil phase with alteration of temperature to compensate for viscosity changes which would normally occur in said oil phase in the absence of said resinous phase.

3. A lubricant comprising a lubricating oil phase and a high molecular weight resinous phase, said resinous phase being less than approximately 0.1% soluble in the lubricating oil phase at a temperature within the range of approximately 65° to 100° F. and more than approximately 1% soluble therein at a temperature within the range of approximately 200° to 300° F., whereby said resinous phase goes out of and into solution in said oil phase with alteration of temperature to compensate for viscosity changes which would normally occur in said oil phase in the absence of said resinous phase.

4. A lubricating composition as defined in claim 1, in which said high molecular weight resinous phase comprises a discontinuous phase non-colloidal dispersed in said lubricating oil phase.

5. A lubricating composition as defined in claim 1, in which said high molecular weight resinous phase comprises a macroscopic dispersion in said lubricating oil phase.

6. A lubricating composition as defined in claim 1, in which said high molecular weight resinous phase comprises a resinous material dissolved in a high boiling solvent immiscible with the oil when cold.

7. A lubricating composition as defined in claim 1, in which said high molecular weight resinous phase comprises a resinous material dissolved in a high boiling solvent immiscible with the oil when cold but miscible therewith when hot.

8. A lubricating composition as defined in claim 1, in which said high molecular weight resinous phase comprises a colloidal dispersion of a resinous material in a dispersing medium other than the lubricating oil, said dispersing medium being substantially insoluble in said lubricating oil when cold.

9. A lubricating composition as defined in claim 1, in which said high molecular weight resinous phase comprises a colloidal dispersion of a resin-

ous material in a dispersing medium other than the lubricating oil, said dispersing medium being substantially insoluble in said lubricating oil when cold but substantially soluble therein when hot.

10. A system for lubricating machine parts comprising a lubricating oil phase, a normally liquid second phase containing a resinous organic material comprising long chain molecules and adapted to increase the viscosity of said lubricating oil when dissolved therein, said resinous material being at least largely insoluble in said oil at approximately 65° F. and at least largely soluble in said oil at approximately 300° 15 F., a normally fluid third phase comprising a low molecular weight fluid adapted to materially decrease the viscosity of said lubricating oil when dissolved therein, said fluid being soluble in said lubricating oil at 65° F. and substantially less 20 soluble in said lubricating oil at 300° F., and means for contacting said lubricating oil with each of said phases in at least one point in said system, whereby said resinous material is dissolved in said oil and said low molecular weight 25 fluid goes out of solution from said oil as the temperature thereof approaches 300° F., and whereby said resinous material is precipitated from solution and said low molecular weight fluid is dissolved in said oil as the temperature thereof approaches 65° F.

11. A method of maintaining the viscosity of a lubricating oil phase within predetermined limits over a temperature range of at least approximately 100° F., which comprises contacting said oil as a first phase with a second phase containing a high molecular weight resinous material substantially insoluble in said oil at the lower temperature of said range, dissolving the resinous material in the oil phase as the temperature 35 progressively rises through said range, and precipitating the resinous material from the oil phase as the temperature of the oil is lowered progressively through said range.

12. A lubricant comprising a continuous lubricating oil phase selected from the group consisting of animal and vegetable oils and a second phase comprising a high molecular weight isobutene polymer substantially insoluble in said continuous phase when cold and largely soluble 45 therein when hot, whereby said second phase goes out of and into solution in said oil phase with alteration of temperature to compensate for viscosity changes which would normally occur in said oil phase in the absence of said second phase.

13. A lubricant comprising a continuous lubricating oil phase of castor oil and a second phase comprising a high molecular weight isobutene polymer substantially insoluble in said continuous phase when cold and largely soluble therein when hot, whereby said second phase goes out of and into solution in said oil phase with alteration of temperature to compensate for viscosity changes which would normally occur in said oil phase in the absence of said second phase.

14. A lubricant comprising a continuous lubricating oil phase of lard oil and a second phase comprising a high molecular weight isobutene polymer substantially insoluble in said continuous phase when cold and largely soluble therein when hot, whereby said second phase goes out of and into solution in said oil phase with alteration of temperature to compensate for viscosity changes which would normally occur in said oil phase in the absence of said second phase.

15. A lubricant comprising a continuous hydrocarbon lubricating oil phase and a second phase comprising a heavy linseed oil polymer of a gelled or semi-solid consistency, said polymer being soluble in said hydrocarbon oil at elevated temperatures of from approximately 200° to 300° F. and insoluble therein at ordinary atmospheric temperatures, said lubricating oil phase having in the absence of the second phase a viscosity index above approximately 50, whereby said polymer goes out of and into solution in said oil phase with alteration of temperature to compensate for viscosity changes which would normally occur in said oil phase in the absence of said second phase.

16. A lubricant comprising a continuous hydrocarbon lubricating oil phase of mixed butene polymers and a second phase comprising a heavy linseed oil polymer of a gelled or semi-solid consistency, said polymer being soluble in said hydrocarbon oil at elevated temperatures of from approximately 200° to 300° F. and insoluble therein at ordinary atmospheric temperatures, whereby said second phase goes out of and into solution in said oil phase with alteration of temperature to compensate for viscosity changes which would normally occur in said oil phase in the absence of said second phase.

AUGUSTUS H. BATCHELDER.